# EUROPEAN PATENT APPLICATION

(11) **EP 2 034 049 A1**
(43) Date of publication of application: **11.03.2009**
(21) Application number: 07115731.7
(22) Date of filing: 05.09.2007
(51) Int. Cl.: C23C 18/20, C23C 18/16

(54) **An electroless process for depositing a metal on a non-catalytic substrate**

(71) Applicant: Nederlandse Organisatie voor Toegepast- Natuurwetenschappelijk Onderzoek TNO, 2628 VK Delft (NL)
(72) Inventor: Tacken, Roland Anthony, 5663 SH Geldrop (NL); De Zwart, Renatus Marius, 5655 JP Eindhoven (NL); Hovestad, Arjan, 5231 PK 's-Hertogenbosch (NL)
(74) Representative: Hatzmann, Martin

(57) **Abstract**

The invention provides an electroless process for depositing a metal on a non-catalytic substrate, which process comprises the steps of:
(a) providing a non-catalytic substrate; and
(b) exposing the substrate to an electroless solution to deposit the metal on the substrate, which solution comprises metal ions and a reducing agent for reducing the metal ions into the metal, whereby at least the surface of the substrate is heated to a temperature (T1) which is higher than the temperature (T2) of the solution.

## Description

The present invention relates to an electroless process for depositing a metal on a non-catalytic substrate, an electric circuit comprising a substrate obtained with said process, and an electric device comprising such an electric circuit.

Various processes are known to deposit a metal on an object such as for instance a plastic, ceramic or metallic substrate. Such processes include electroplating processes wherein use is made of an electrical current to deposit a metal layer on an electrically conductive object, e.g. substrate. Both the object and the metal component to be deposited on the object are placed in a solution, whereby the object to be plated functions as the cathode and the metal component functions as the anode. The solution contains one or more salts of the corresponding metal together with other ions that allow electricity to flow through the solution. Electricity is supplied to the object to be coated causing the metal ions in the solution to be reduced to the metal which deposits on the object, whereas the metal component dissolves and replenishes its metal ions in the solution. Such an electroplating is used for instance to improve various properties of the object to be coated, e.g. wear resistance and corrosion protection.

Electroless processes constitute another category of processes in which a metal can be deposited on a substrate. Electroless processes depend on the catalytic reduction of metal ions in an aqueous solution which contains a reducing agent which establishes that the metal ions will be reduced to the corresponding metal and deposit on the object to be coated without the use of an external electric current. The deposition of the metal concerned takes place on a catalytic substrate. A few metals have the ability to initiate and catalyze the electroless deposition of a metal on a substrate, e.g. Pd, Ag, Au, Pt, Cu and Ni. Substrates that need to be metallized but that do not consist or contain one of these catalytic metals, are typically made catalytic by adsorption of catalytic colloids to the surface of the substrate. Most often, this is done by absorption of palladium colloids on the surface of the substrate on which the desired metal is to be deposited. In addition to the substrate, the metal to be deposited on the substrate should also be catalytic to the reduction reaction, rendering the process autocatalytic as such. For a general description on electroless plating processes reference can, for instance, be made to Electroless Plating Fundamentals & Applications, edited by Glenn O. Mallory and Juan B. Hajdu, New York (1990*).* When compared with electroplating processes, electroless plating processes have general the advantage that no electrical power is required and that improved metal coatings can be established in terms of uniformity and stress of deposits.

Object of the present invention is to provide an electroless plating process in which no metal catalyst is required to initiate and catalyze the deposition of a desired metal on the surface of a substrate.

Surprisingly, it has now been found that this can be established when the temperature of the surface on which the metal needs to be deposited is higher than the temperature of the solution containing the metal ions and the reducing agent.

Accordingly, the present invention relates to an electroless process for depositing a metal or alloy thereof on a non-catalytic substrate, which process comprises the steps of:
(a) providing a non-catalytic substrate; and
(b) exposing the substrate to an electroless solution to deposit the metal on the substrate, which solution comprises metal ions and a reducing agent for reducing the metal ions into the metal, whereby at least the surface of the substrate is heated to a temperature (T1) which is higher than the temperature (T2) of the solution.

The process according to the present invention has the advantages that no metal catalyst needs to be applied on the substrate surface to initiate and catalyze the metallization process. Moreover, metal deposition is rapid because of the high temperatures applied. Hence, in the context of the present invention, a non-catalytic substrate is a substrate on which no metal catalyst has been applied to initiate or catalyze the deposition of a metal or alloy thereof on its surface.

The substrate can be exposed to the electroless solution in various ways. For instance, the electroless solution can be brought into contact with the non-catalytic substrate by means of an inkjet printing process, the substrate can be immersed in the electroless solution or, in case the substrate has the form of a moulded product, the electroless solution can be brought into contact with the moulded product in the mould in which the moulded product has been or is being produced.

Preferably, the non-catalytic substrate is immersed in the electroless solution comprising the metal ions and the reducing agent.

Suitably, the metal or alloy to be deposited on the non-catalytic substrate is selected from the group consisting of nickel, copper, gold, silver, tin, or any alloy thereof, and nickel-boron and nickel-phosphorous,.

Preferably, the metal to be deposited on the non-catalytic substrate is copper. Preferably, the alloy to be deposited on the non-catalytic substrate is nickel-phosphorous or nickel-boron alloy.

In accordance with the present invention, at least the surface of the substrate is heated to a temperature (T1) which is higher than the temperature (T2) of the solution.

Suitably, the temperature T1 is in the range of from 50-200°C. Preferably, the temperature T1 is in the range of from 80-180°C, more preferably in the range of from 70-140°C.

Suitably, the temperature T2 is in the range of from 15-90°C. Preferably, the temperature T2 is in the range of from 15-60°C. More preferably in the range of from 15-25°C In other words, T2 can suitably be the ambient temperature.

The non-catalytic substrate to be used in accordance with the present invention can suitably comprise liquid crystalline polymer (LCP), polyamide, polyethyleneimine (PEI), acrylonitrile-butadiene-styrene (ABS), polycarbonate/ABS, or a thermohardening material such as an epoxy or polyester compound.

In the process according to the present invention the concentration of both the metal ions and reducing agent present in the electroless solution are generally chosen as high as possibly, i.e. close to maximum solubility, while maintaining room temperature stability.

The reducing agent to be used in accordance with the present invention can suitably selected from the group consisting of formaldehyde, dimehtylaminoborane, hypophosphite, sodium borohydride and hydrazine.

The electroless solution to be used in the present process can suitably further comprise a complexing agent. Said complexing agent can suitably be selected from the group consisting of acetate, propionate, succinate, hydroxyacetate, ammonia, hydroxypropionate, glycolic acid, aminoacetate, ethylenediamine, aminopropionate, malonate, pyrophosphate, malate, citrate, gluconate, tartate, EDTA, proprionitrile, tetraethylenetetraamine, 1,5,8,12 tetraazaundecane, 1,4,8,12 tetraazacyclopentadecane, and 1,4,8,11 tetraazandecane.

The electroless solution to be used in accordance with the present invention can suitably further comprise a buffering agent. Said buffering agent can suitably be selected from the group consisting of acetic acid, propionic acid, succinic acid, glutaric acid, adipic acid, organic amines, and carboxylic acids.

The electroless solution to be used in the present process can suitably further comprise a stabilizer. Said stabilizer may suitably comprise heavy metal ions, an organic or inorganic sulphur, selenium or tellur-containing compound.

In a particular embodiment, the present process is carried out in a mould, and whereby the substrate is formed in the mould by means of a three-dimensional injection moulding process.

In addition, the present invention also relates to an electric circuit which comprises an substrate as obtained with the present process.

The present invention also relates to a device comprising a substrate as obtained in accordance with the present invention.

Suitable devices include, but are not limited to, antenna structures, interconnection elements sensors, and actuators.

Preferably, the device according to the present invention is an electric device which comprises an electric circuit in accordance with the present invention.

### Example

A electroless plating solution was used which contained copper sulfate in an amount of 0.06 mol/l. The electroless solution was buffered using triethanolamine in a concentration of 0.2 mol/l. The pH of the electroless solution was 9.0. The electroless solution so obtained was then is stabilised using 1,4,8,11 tetraazaundecane as a complexing agent in an amount of 0.05 mol/l. The electroless solution further contained as the reducing agent dimethylaminoborane in an amount of 0.06 mol/l. The electroless solution having an ambient temperature was then brought in contact with a polyamide substrate (type Stanyl TE200F6, supplier DSM) having on the surface a temperature of 130°C. A closed metallised electrically conducting surface was obtained within 20 seconds.

## Claims

1. An electroless process for depositing a metal on a non-catalytic substrate, which process comprises the steps of:
(a) providing a non-catalytic substrate; and
(b) exposing the substrate to an electroless solution to deposit the metal on the substrate, which solution comprises metal ions and a reducing agent for reducing the metal ions into the metal, whereby at least the surface of the substrate is heated to a temperature (T1) which is higher than the temperature (T2) of the solution.

2. A process according to claim 1, wherein the substrate is immersed in the solution.

3. A process according to claim 1 or 2, wherein the metal is selected from the group consisting of copper, nickel, gold, silver, tin, or any alloy thereof, and nickel-boron and nickel-phosphorous.

4. A process according to claim 3, wherein the metal is copper.

5. A process according to claim 3, wherein the alloy is nickel-phosphorous or nickel-boron.

6. A process according to any one of claims 1-5, wherein the temperature T1 is in the range of from 50-200°C.

7. A process according to claim 6, wherein the temperature T1 is in the range of from 70-140°C.

8. A process according to any one of claims 1-7, wherein the temperature T2 is in the range of from 15-90°C.

9. A process according to claim 8, wherein the temperature T2 is in the range of from 15-25°C.

10. A process according to any on of claims 1-9, wherein the substrate comprises liquid crystalline polymer (LCP), polyamide, polyethyleneimine (PEI), acrylonitrile-butadiene-styrene (ABS), polycarbonate/ABS, or a thermohardening material such as an epoxy or polyester compound.

11. A process according to any one of claims 1-10, wherein the reducing agent is selected from the group consisting of formaldehyde, dimehtylaminoborane, hypophosphite, sodium borohydride and hydrazine.

12. A process according to any one of claims 1-11, wherein the solution further comprises a complexing agent.

13. A process according to claim 12, wherein the complexing agent is selected from the group consisting of acetate, propionate, succinate, hydroxyacetate, ammonia, hydroxypropionate, glycolic acid, aminoacetate, ethylenediamine, aminopropionate, malonate, pyrophosphate, malate, citrate, gluconate, tartate, EDTA, proprionitrile, tetraethylenetetraamine, 1,5,8,12 tetraazaundecane, 1,4,8,12 tetraazacyclopentadecane, and 1,4,8,11 tetraazandecane.

14. A process according to any one of claims 1-15, wherein the solution further comprises a buffering agent.

15. A process according to claim 14, wherein the buffering agent is selected from the group consisting of acetic acid, propionic acid, succinic acid, glutaric acid, adipic acid, organic amines, and carboxylic acids.

16. A process according to any one of claims 1-15, wherein the solution further comprises a stabilizer.

17. A process according to claim 16, wherein the stabilizer comprises heavy metal ions, an organic or inorganic sulphur, selenium or tellur-containing compound.

18. A process according to any one of claims 1-17, which is carried out in a mould, and whereby the substrate is formed in the mould by means of a three-dimensional injection moulding process.

19. An electric circuit which comprises a substrate as obtained according to any one of claims 1-18.

20. An electric device which comprises an electric circuit according to claim 19.
